

## UNITED STATES PATENT OFFICE

2,657,984

## FUEL OILS

Charles Henry Braithwaite, Jr., Wood River, and George Ambrose Martin and Reid Edward Sutton, East Alton, Ill., assignors to Shell Development Company, San Francisco, Calif., a corporation of Delaware

No Drawing. Application October 20, 1950,  
Serial No. 191,332

11 Claims. (Cl. 44—71)

1

This invention relates to petroleum fuels and, more particularly, to novel fuel oil compositions having greatly improved pour-point characteristics.

One of the characteristics of fuel oils which is limited by standardized specifications is the property known as "pour-point." Because of this requirement that fuel oils have a specified minimum pour point, rather severe limitations are inherently placed upon the relative quantities of gasolines, light distillate oils, residual fuels, etc., which may be produced from a given crude petroleum stock. For example, in order to meet the pour-point specification, a distillate furnace oil must contain a certain proportion of fairly light components, or cannot contain more than a certain proportion of heavy components. If, however, the pour point of the fuel is reduced in some manner, a smaller proportion of the volatile components is required in the furnace oil, and larger quantities of lighter distillates such as kerosene and gasoline can be produced. Likewise, during periods of peak demand for fuel oils, greater quantities of such oils can be produced by including therein larger amounts of heavier fractions. Other beneficial results of a suitable means of lowering the pour point of fuel oils will be obvious to those skilled in the art.

It has now been found that the pour point of a petroleum fuel oil may be lowered by the inclusion of small amounts of a compound containing the structural group,



(1)

where X is a chalcogen or an NH group. It will be noted that the above formula gives one a wide choice of satisfactory materials, the only limitation being that the compound should have a solubility in the oil greater than about 0.0005 per cent by weight, and preferably greater than about 0.001 per cent by weight. A particularly effective embodiment of the invention is obtained when the bond on the carbon atom in Formula 1 is satisfied by an amino or substituted amino group and X is an oxygen or sulfur atom. These ureas,



(2)

may have either hydrogen atoms or organic radicals attached to the nitrogen atoms, but because of the requirement as to oil solubility, at least one oil-solubilizing hydrocarbon radical will generally be necessary to make the compound suffi-

2

ciently soluble in most fuel oils. The preferred organic radicals are hydrocarbon radicals, which may be aliphatic or cyclic, straight or branched chain, saturated, unsaturated or aromatic or any combination thereof. Thus, the hydrocarbon radicals may be, for example, alkyl, alkenyl, aryl, alkaryl, aralkyl, etc.

The ureas may be substituted with other than pure hydrocarbyl radicals. For example, the hydrocarbyl radical may be substituted with amino, hydroxy, alkoxy, aryloxy, carboxylate, oxo, halogen, or like substituents; or the nitrogen of the urea may be directly attached to a non-carbon atom, such as another nitrogen atom, to form semicarbazides, semicarbazones, and the like.

While the ureas are the preferred embodiment of the present invention, non-urea materials having the structure of Formula 1 may be used if desired. For example, amides or substituted amides, carbamates, amidines such as guanidine or stearamidine, etc., are all effective, provided the solubility requirement is met. Likewise, combinations of the above essential structure may be used, as in biuret, or derivatives thereof.

The foregoing describes in relatively general terms the structural requirements and physical properties of the additives of the present invention. For specific examples of satisfactory compounds, reference may be had to the tables presented below. The data therein were obtained by measuring the pour points (determined according to ASTM Specification D-97-47 except that observations were made at temperature intervals of 2° F. rather than 5° F., and two or more determinations were made on each specimen and the average result reported) of a Number 2 fuel oil (ASTM Specification D-396-39T), with and without the various pour-point depressants of this invention.

The No. 2 fuel has the following properties:

|                               |                              |
|-------------------------------|------------------------------|
| Flash point, °F-----          | Minimum 110,<br>maximum 190. |
| Pour point, °F-----           | 10.                          |
| Water and sediment, per cent  | 0.05.                        |
| Carbon residue, per cent----- | 0.25 and 10% residual.       |
| Distillation temperature, °F: |                              |
| 10% point-----                | 440.                         |
| 90% point-----                | Maximum 600.                 |

Unless otherwise noted, the pour-point depressant was used at a concentration of 0.0015 per cent by weight.

### 3 Table I

| Compound                                                           | Pour-point<br>Depression,<br>°F. |
|--------------------------------------------------------------------|----------------------------------|
| Phenylthiourea                                                     | 4                                |
| Oleoylurea                                                         | 3                                |
| Stearylurea (at 0.0075% weight)                                    | 3                                |
| Cyclohexylurea                                                     | 4                                |
| Dodecylurea                                                        | 4                                |
| Ethyliureidoacetate                                                | 3                                |
| alpha-Phenyl ethylurea                                             | 4                                |
| alpha-Phenyldodecylurea                                            | 10                               |
| p-Dimethylaminophenylurea                                          | 3                                |
| Dibenzylurea                                                       | 3                                |
| N-Dodecyl-N'-phenylthiourea                                        | 4                                |
| N-Phenyl-N-n-butyl-N'-phenylthiourea                               | 3                                |
| N-Cyclohexyl-N'-phenylthiourea                                     | 3                                |
| N,N-Dicyclohexyl-N'-phenylurea                                     | 3                                |
| Phenylurethane of 5-hydroxymethyl-2,2,4,8,10,10-hexamethylundecane | 4                                |
| 3,5,5-Trimethylhexylurea                                           | 5                                |

Other materials which depressed the pour point of fuel oils when present at a concentration of 0.0015 wt. percent are listed in Table II.

Table II.

-Di-n-butylthiourea  
 -s-Di-n-butylurea  
 -tert-Amylurea  
 -Stearoylurea  
 -Undecylenoylurea  
 -Benzylurea  
 -Octylurea  
 -2-methyl-5-isopropylphenylurea  
 -2,6-dimethyl-4-heptylurea  
 -Diisobutylketone semicarbazone  
 -N-phenyl-N-methyl-N'-phenylthiourea  
 -N-phenyl-N-ethyl-N'-phenylthiourea  
 -N-phenyl-N-n-propyl-N'-phenylthiourea  
 -N,N-diethyl-N'-phenylthiourea  
 -N-cyclohexyl-N-amyl-N'-phenylthiourea  
 -N-di-2-ethylhexyl-N'-phenylthiourea  
 -N-stearyl-N'-phenylthiourea  
 -N-benzyl-N'-phenylthiourea  
 -N,N-di-n-amyl-N'-phenylthiourea  
 -N,N-diisoamyl-N'-phenylthiourea  
 -N-dodecyl-N'-phenylurea  
 -N-stearyl-N'-phenylurea  
 -N-cyclohexyl-N-amyl-N'-phenylurea  
 -N,N-(di-2-ethylhexyl)-N'-phenylurea  
 -N,N-dibenzyl-N'-phenylurea  
 -N-cyclohexyl-N-phenyl-N'-phenylurea  
 -Phenylurethane of sec-butylalcohol  
 -Phenylurethane of n-hexylalcohol  
 -Phenylurethane of n-decylalcohol  
 -N-(alpha-phenylethyl)-N'-phenylurea  
 -as-Diphenylurea  
 -N,N,N',N'-tetra-n-butylurea  
 -as-Di-n-octylurea  
 -N-(2-ethylhexyl)-N'-phenylurea  
 -N-(3,5,5-trimethylhexyl)-N'-phenylurea  
 -N-alpha-phenyldodecyl-N'-phenylurea  
 -Gamma-2-ethylhexoxy propylurea  
 -2-ethylhexylurea  
 -N-phenyl-N-ethyl-N'-octadecylurea  
 -N-phenyl-N-n-propyl-N'-octadecylurea  
 -N-phenyl-N-n-butyl-N'-octadecylurea  
 -s-Dioctadecylurea  
 -N-benzyl-N-phenyl-N'-octadecylurea  
 -N-(gamma-(2-ethylhexoxy)-propyl)-octadecylurea  
 -Ester of N-octadecylcarbamic acid and  
 -droxymethyl-2,2,4,8,10,10-hexamethyl  
 -ane  
 -N-alkylamine\*-N'-octadecylurea  
 -N-benzyl-N-phenyl-N'-phenylurea

The importance of oil solubility may be seen from the following data comparing the effects of adjacent homologues.

Table III.-

| Compound                          | Pour-Point Depression, °F. |
|-----------------------------------|----------------------------|
| Phenylurea                        | 1                          |
| N-Phenyl-N-methylurea             | 2                          |
| N-Phenyl-N-ethylurea              | 2                          |
| N-Phenyl-N-n-propylurea           | 5                          |
| N-Phenyl-N-methyl-N'-phenylurea   | 2                          |
| N-Phenyl-N-ethyl-N'-phenylurea    | 4                          |
| N-Phenyl-N-n-propyl-N'-phenylurea | 5                          |
| N-Phenyl-N-n-butyl-N'-phenylurea  | 6                          |

The above pour-point depressants may be used alone or in conjunction with other pour-point depressants.

20 The above pour-point depressants may be effectively utilized in fuel oils, either residual or distillate, but are particularly effective in the latter. The distillate fuel oils, variously called "furnace oils," "gas oils," "burner fuels" and the like, may be characterized as relatively unrefined distillate fuels of rather high boiling point range. Such fuels usually have an initial boiling point higher than about 350° F. or 375° F., and the final boiling point often is in excess of 30 700° F. The sulfur content generally will be in excess of 0.1%, as will be the carbon residue (Ramsbottom). Typical domestic fuel oils are often made up of blends of catalytically cracked gas oils and straight-run distillates, while an industrial furnace oil may be made up entirely of catalytically cracked gas oil fractions.

The most effective concentration of the pour-point depressant, and the amount of depression obtained, may vary from one fuel oil to the next, but, in general, the optimum concentration will be between about 0.0005 wt. percent and about 1.0 wt. percent of the depressant in the oil, or even between about 0.001% and about 0.1%.

When the depressants of this invention are used in conjunction with another material, they will usually be used in amounts of between about 0.005 and about 2% by weight of the oil.

The invention claimed is:

1. A distilled fuel oil having an initial pour-point of at least about  $10^{\circ}$  F. containing dissolved therein a minor but effective pour-point depressing amount of a metal-free compound having the formula.



wherein R is an alkyl radical, said compound having a solubility greater than about 0.001 per cent by weight in said fuel oil.

60 2. A distillate fuel oil having an initial pour-point of at least about 10° F. containing dissolved therein a minor but effective pour-point depressing amount of a metal-free compound having the formula, 3.



70 wherein R is a hydrocarbyl radical and X is a chalkogen having an atomic number of from 8 to 16, said compound having a solubility greater than 0.0005 per cent by weight in said fuel oil.

3. A distillate fuel oil having an initial pour-point of at least about 10° F. containing distillate having a minor but effective pour-point

\* Mixture of C<sub>12</sub>-C<sub>15</sub> highly branched primary amines.

depressing amount of a metal-free compound having the formula,



wherein  $R_1$  is a hydrocarbyl radical and  $R_2$  is selected from the group consisting of hydrogen atoms and hydrocarbyl radicals.

4. A distillate fuel oil having an initial pour point of at least about  $10^{\circ}$  F. containing dissolved therein a minor but effective pour-point depressing amount of a metal-free compound having the formula,



wherein  $R_1$  is a hydrocarbyl radical and  $R_2$  is selected from the group consisting of hydrogen atoms and hydrocarbyl radicals.

5. A fuel oil having an initial pour point of at least about  $10^{\circ}$  F. containing dissolved therein a minor but effective pour-point depressing amount of a metal-free compound having the formula,



wherein  $R_1$  is a hydrocarbyl radical,  $R_2$  is selected from the group consisting of hydrogen atoms and hydrocarbyl radicals, and  $X$  is a chalkogen having an atomic number of from 8 to 16.

6. A fuel oil having an initial pour point of at least about  $10^{\circ}$  F. containing dissolved therein a minor but effective pour-point depressing amount of a metal-free compound having the structural group,



wherein  $X$  is a chalkogen having an atomic number of from 8 to 16, said compound having at least one hydrocarbyl group attached to a nitrogen atom.

7. A distillate fuel oil having an initial pour point of at least  $10^{\circ}$  F. containing a minor but effective pour-point depressing amount of lauryl urea dissolved therein in amount greater than 0.0005% by weight and not greater than 1.0% by weight.

8. A distillate fuel oil having an initial pour point of at least  $10^{\circ}$  F. containing a minor but effective pour-point depressing amount of N-phenyl - N - n - butyl - N' - phenylurea dissolved therein in an amount greater than 0.0005% by weight and not greater than 1.0% by weight.

9. A distillate fuel oil having an initial pour point of at least  $10^{\circ}$  F. containing a minor but effective pour-point depressing amount of N-phenyl - N - n - propyl-N'-phenylurea dissolved therein in an amount greater than 0.0005% by weight and not greater than 1.0% by weight.

10. A distillate fuel oil having an initial pour point of at least  $10^{\circ}$  F. containing a minor but effective pour-point depressing amount of phenylthiourea dissolved therein in an amount greater than 0.0005% by weight and not greater than 1.0% by weight.

11. A distillate fuel oil having an initial pour point of at least  $10^{\circ}$  F. containing a minor but effective pour-point depressing amount of stearylurea dissolved therein in an amount greater than 0.0005% by weight and not greater than 1.0% by weight.

CHARLES HENRY BRAITHWAITE, JR.  
GEORGE AMBROSE MARTIN.  
REID EDWARD SUTTON.

References Cited in the file of this patent  
UNITED STATES PATENTS

| Number    | Name     | Date          |
|-----------|----------|---------------|
| 2,263,445 | Reiff    | Nov. 18, 1941 |
| 2,343,393 | Bergen   | Mar. 7, 1944  |
| 2,373,049 | Pedersen | Apr. 3, 1945  |
| 2,393,934 | Reiff    | Jan. 29, 1946 |
| 2,396,156 | Clarkson | Mar. 5, 1946  |

## FOREIGN PATENTS

| Number  | Country       | Date         |
|---------|---------------|--------------|
| 312,774 | Great Britain | June 6, 1929 |